# EUROPEAN PATENT SPECIFICATION

(11) **EP 0 086 988 B1**
(45) Date of publication and mention of the grant of the patent: **08.04.1987**
(21) Application number: 83100777.8
(22) Date of filing: 27.01.1983
(51) Int. Cl.: C21D 9/08

(54) **Method and apparatus for quenching steel pipes**
Verfahren und Vorrichtung zum Abschrecken von Stahlrohren
Procédé et appareil pour tremper des tubes en acier

(30) Priority: 08.02.1982 US 346755
(43) Date of publication of application: 31.08.1983
(73) Proprietor: KRUPPERT ENTERPRISES, INC., Goulais River Ontario POS 1EO (CA)
(72) Inventor: Kruppert, Frederick, William, Goulais River Ontario POS 1EO (CA)
(74) Representative: Grünecker, Kinkeldey, Stockmair & Schwanhäusser Anwaltssozietät

## Description

The present invention relates to an apparatus and method for hardening steel and more particularly to a method and apparatus for quenching steel pipes of substantial and varying thicknesses.

Quenching is one of the oldest and most common methods of hardening steel by heat treatment. It consists of heating the steel above its critical transformation temperature at which a component known as austenite begins to form, and then cooling it fast enough, usually by quenching into a liquid such as water or oil, to avoid any transformation of the austenite until it reaches the relatively low temperature range within which it transforms to a hard martensite. The steel is subsequently reheated or tempered to remove the internal stresses caused by the inherent expansion of the martensite.

The quenching of steel from its critical transformation temperature to the martensitic transformation temperature requires a rather severe cooling rate if the formation of pearlite is to be avoided. Given the importance of the cooling rate in producing the desired properties, the production of large pieces of steel has always presented particular difficulties, since the temperature drop at the center of a given piece of steel lags the temperature drop at the surface.

A number of processes have been developed in an attempt to address this problem. For example, metal alloys, such as manganese, silicon, nickel or chromium have been added to retard the formation of pearlite to allow for an initial lower quench and to enhance in other ways the final properties of the steel. However, the use of alloys adds considerably to the expense of the steel.

A variety of methods and devices have been developed or suggested as ways of more readily controlling heat transfer from both the exterior and interior surfaces of pipes by using water, as well as other substances, as a cooling medium. These prior processes employ a variety of sprays and flow schemes. For example, in U.S. Patent No. 3,212,766 there is disclosed a generic apparatus for quenching a long tube. Said conventional apparatus comprises a quenching receptacle adapted to receive a tube and a cooling medium. A cooling medium source for supplying the cooling medium is also shown in the citation and said cooling medium source comprises an exterior quenching means in the form of an oil bath. The conventional apparatus, however, fails to provide a sufficiently severe quench so that the thickness of steel pipe which may be successfully treated is limited. Furthermore, said conventional apparatus appears to be unable to provide uniform cooling or to accommodate a steel piece of varying thickness such as upset pipe.

U.S. Patent No. 3,623,716 discloses an apparatus for hardening long pipes. The pipe is immersed in a tank equipped with a nozzle arranged for introducing a cooling medium into the interior of the pipe in such a manner that cooling medium is drawn from the exterior of the pipe to the interior of the pipe.

U.S. Patent No. 3,877,685 discloses an apparatus for quenching a steel pipe with a cooling medium including an isolator which is in fluid communication with a retractable nozzle. The isolator and retractable nozzle cooperate so that the relative proportion of cooling liquid passing into the pipe and around the pipe may be varied. The flow of cooling medium is directed along the longitudinal axis of the steel pipe.

U.S. Patent No. 4,165,246 discloses a process for heat treating steel pipes with a wall thickness ranging from 16 to 36 mm. After the steel pipe is heated, it is passed on rollers to a cooling zone while water directed from nozzles encircling the pipe quench the surface below the martensitic transformation temperature.

U.S. Patent No. 4,116,716 discloses an immersion cooling apparatus including a cooling tank containing cooling liquid, a mechanism for locking the immersed pipe in position, and a nozzle extending toward the interior of the pipe in the direction of the pipe axis.

It is, therefore, an object of the invention to provide a quenching apparatus according to the precharacterising part of claim 1 enabling a more severe quench for a given thickness of steel.

The above object of the present invention is achieved by the invention as defined in claim 1.

Concerning a method of heat treating pieces of steel including the step of heating each piece of steel to a temperature above its austenizing temperature, the object of the present invention is achieved by the subject matter of claim 12.

As to improvements obtainable by the claimed features, generally in the apparatus and method according to the invention, the use of a continually replenished cooling medium in a circumferential flow pattern provides an improved control of temperature and so allows a more severe quench-for a given thickness of steel. This in turn can improve the properties of the steel or allow reduction in the alloys necessary to obtain particular properties in a piece of steel. The necessity for continually replenishing the cooling medium once it has removed heat from the pipe or other piece of steel to be quenched is in part illustrated by the loss of cooling power in water. For example, water at a temperature of 100°F (49°C) has only about 20% of the cooling power of water at 70°F (21°C). Also, continual replenishment of the cooling medium facilitates the removal of impurities.

Further, the use of a circumferentially variable flow rate allows the uniform quenching of pieces of steel of varying shape or thickness. Thus, the apparatus or method according to the invention may be readily adapted to quench upset pipe.

The use of an internal quench is also important in that it promotes a more uniform cooling sequence across the thickness of a steel pipe. It is believed that the use of a gas with water at sufficient pressure will force the water to adhere more closely to the interior pipe wall as it passes through the pipe and so promote more uniform cooling.

Claims 2 to 11 and 13 to 17 contain advantageous embodiments of the apparatus and method according to the invention, respectively.

Examples of the more important features of this invention have thus been summarized rather broadly in order that the detailed description thereof that follows may be better understood, and in order that the contribution to the art may be better appreciated. There are, of course, additional features of the invention that will be described hereinafter and which will also form the subject of the claims appended hereto.
Figure 1 is a plan view of a preferred embodiment of the present invention;
Figure 2 is an elevation view of the embodiment depicted in Figure 1;
Figure 3 is a closeup view of a portion of the embodiment shown in Figure 2;
Figure 4 is a closeup view of a portion of the embodiment of Figures 1, 2, and 7, taken along line 4-4 of Figure 7;
Figure 5 is a cross sectional view taken along line 5-5 in Figure 1;
Figure 6 is a cross sectional view of another embodiment of the present invention;
Figure 7 is another cross sectional view taken from Figure 1 along line 7-7;
Figure 8 is a vertical cross sectional view of a portion of an internal quenching means;
Figure 9 is a partial cross sectional frontal view taken along line 9-9 from Figure 8; and
Figure 10 is a closeup view of gas conduit outlet of the internal quenching means.
Reference to these drawings will further explain the invention when taken in conjunction with the description of the preferred embodiments.

### Description of the Preferred Embodiments

Referring generally now to Figures 1-10, there will now be described a device and method of quenching steel pipe in accordance with the present invention. Generally, the apparatus may include a feed mechanism 10, a pipe receptacle 30, an unloading mechanism 40, a cooling medium source 50, an exterior quenching means 70, an internal quenching means 80, and a clamp 100.

The feed mechanism 10 is adapted to place a pipe 130 into receptacle 30, which is adapted to hold the pipe in place in conjunction with clamp 100. Exterior quenching means 70 is connected to cooling medium source 50 and adapted to direct a cooling medium such as water in a substantially circumferential flow pattern around exterior segments of the pipe in the receptacle. The exterior quenching means 70 may be adapted in conjunction with cooling medium source 50 to provide variable flow rates to differing segments of the pipe. Internal quenching means 80 is also connected to a cooling medium source and is adapted to concurrently pass a cooling medium through the interior of the pipe as it is in the receptacle. Interior quenching means 80 includes means for injecting a gas into the cooling medium to insure sufficient turbulence in the cooling medium as it passes through the pipe to facilitate heat transfer from the pipe to the cooling medium.

Referring now to Figures 1 and 7 feed mechanism 10 comprises feed rolls 11. The feed rolls are each mounted on feed roll shafts 12 which are in turn journaled into jaws 13 mounted on base 14. A hydraulic cylinder 17 is pivotally mounted by means of pin 16 to base 15. Piston 18 of hydraulic cylinder 17 is connected at one end to flange or arm 27 which rotates on shaft 21. As best shown in Figure 1, flange 27 is integrally but separately mounted to shaft 21 such that movement of piston 18 causes movement of flange 27 and so rotation of shaft 21.

A number of angular feed arms 22 are also integrally mounted along shaft 21. Each anagular feed arm 22 has an arcuate portion 24 which is adapted to cradle the largest pipe to be heat treated. As best shown in Figure 7, arms 22 are mounted such that when piston 18 is extended arcuate portion 24 of angular feed arm 22 is sufficiently below the level of feed rolls 11 to allow passage of the pipe along the feed rolls.

The angular feed arms 22 are adapted to rotate about shaft 21 such that upon rotation of shaft 21 the arcuate portion 24 of the angular feed arm cradles and lifts the pipe off of feed rolls 11 and onto feed ramps 23.

Each feed ramp 23 is mounted at one end on pedestal 28 of post or support 19 and at the other end on pedestal 26 of support 25. As shown in Figure 7, the feed ramp 23 is inclined toward the pipe receptacle indicated generally at 30 so as to facilitate the transfer of the pipe from feed rolls 11 into receptacle 30.

Pipe receptacle 30 comprises a U-shaped exterior wall 34 and a U-shaped interior wall 35 which serve to form an annulus 36 as best shown in Figures 5-7. The walls 34 and 35 extend the length of the receptacle 30. However, as indicated in Figures 1 and 5-7, the annulus 36 is segmented by walls 71 which run along the length of the receptacle 30 and extend radially from walls 34 or 134. Additionally, as shall hereinafter be more fully described, the annulus 36 is further divided along the length of the pipe receptacle 30 by partitions extending from wall 34 and 134 to wall 35. Walls 71 and the partitions in conjunction with walls 34 or 134 and 135 form exterior flow chambers 73.

As shown in Figures 5 and 7, the upper portion of walls 34 and 35 closest to unloading mechanism 40 is lower than the upper portion of wall 35 closest to feed mechanism 10. This arrangement allows excess cooling medium collecting in receptacle 30 to readily spill over the rim of wall 35 on the side opposite the unquenched pipe. The difference in height between the upper wall portions should be sufficient to allow the easy discharge of the cooling medium from receptacle 30. A trough (not shown) may be provided along the length of the receptacle to facilitate removal of the cooling medium as it spills over wall 35.

Interior U-shaped wall or surface 35 is provided with a number of ribs or quenching supports 31 along its length. Each rib 31 is mounted on interior wall 35 by means of rib flanges 37 which are integrally mated to wall 35. Bolts 38 serve to secure rib 31 to the flanges. As best shown in Figure 1, at least the upper portion of each rib 31 is relatively narrow, such that only a minimal portion of the exterior surface of pipe 130 is in contact with the ribs 31 as the pipe rests on the ribs.

As shown in Figure 7, the portions of wall 35, rib 31 and rib flanges 37 nearest feed mechanism 10 are each fixedly attached to each other such that they form a stationary member 32. The remaining portion of wall 35 is attached to interior curved wall 134 by means of side wall 171 and a portion of movable support 49 indicated at 149. Interior curved wall 134 rests on, but is not connected to, exterior wall 34. Thus, the remaining portions of wall 34, rib 31, and rib flange 37 form a movable arm33 which is attached to and movable with movable support 49. As a portion of wall 35 forms an upper surface of movable arm 33 and stationary member 32, the movable arm 33 is flush with the surface of the receptacle 30 except for quenching support 31 and flanges 37.

Pipe receptacle 30 thus comprises an exterior wall 35 with a series of stationary portions or members 32 which are mounted on the side of the receptacle nearest the feed mechanism 10, and a series of juxtaposed movable segments or arms 33, each of which is located opposite a stationary member 32. Each movable arm 33 is provided with an arcuate section 34 which extends across the longitudinal axis of the receptacle 30 such that the pipe 130 is cradled in the arcuate section 34 when' the pipe rests on ribs or quenching supports 31. The movable arms 33 in conjunction with stationary members 32 form partitions. These partitions serve to divide receptacle 30, including annuli 36, into compartments.

Although pipe receptacle 30 is generally illustrated as comprising U-shaped walls, the shape of receptacle 30 may be varied. By way of example, receptacle 30 might be more circular in shape as shown in Figure 6 or might be rectangular or orthogonal along its cross-section. However, U-shaped or curved walls which roughly conform to the shape of the pipe being quenched are preferred for steel pipe, since the curvature of the walls assists in providing a circumferential flow about the exterior of the steel pipe.

The unloading mechanism 40 includes a hydraulic cylinder 43 which is pivotally mounted on base 42 by means of pin 44 and flanges 45. Hydraulic cylinder 43 is equipped with a piston 46 which is connected to arm 48 by means of pin 47. As shown in Figure 1, arm or flange 48 is integrally mounted to shaft 38 such that the movement of arm 48 causes the rotation of shaft 38.

Each movable support 49 is pivotally mounted on base 37 by means of shaft 38, which, as shown in Figure 1, extends substantially the length of receptacle 30. As each movable support 49 is integrally mounted on shaft 38, rotation of shaft 38 causes the movement of each movable support 49. Movable arm 33 is in turn integrally mounted to the upper portion of movable support 49 by means of common wall 149. Thus, movement of piston 46 by hydraulic cylinder 43 causes the movement of movable arm 33 and hence pipe 130 from pipe receptacle 30 to ramp 41. Unloading mechanism 40 is also equipped with rollers 39 to facilitate movement of pipes from ramp 41 for further treatment.

In an alternate embodiment as shown in Figure 6, shaft 38 could be mounted on the upper portion of post 49, thus dividing post 49 into a fixed lower portion integrally attached to base 37 and a pivotal upper portion 149 attached to movable arm 33.

As shown in Figures 5 and 6, the cooling medium source 50 comprises a series of pipes and valves adapted to supply a sufficiently pressurized cooling medium into flow chambers 73 formed in annulus 36 bywalls71 and portions of walls 34 and 35 or 134 and 35. Pipes 55 and 56 branch off from main feed pipe 51 to provide water or other appropriate quenching medium to the exterior quenching system 70. Valves 52 are provided to control the flow rate of the cooling medium to any given flow chamber 73. Although shown as being manually controlled, valves 52 may be linked to appropriate process controls.

The branch pipes 55 and 56 are located between each of the ribs 31 such that the flow of cooling medium may be varied in between divisions formed by stationary members 32 and movable arm 33. Thus, as shall hereinafter be more fully described the flow of cooling medium to any given segment of the exterior surface of pipe 130 may be varied since the flow rate and pressure of the cooling medium to each quenching compartment formed by stationary members 32 and movable arms 33 may be varied by means of valves 52.

Alternately, a greater number of branch pipes may be provided to vary flow of the quenching medium within any compartment. However, in accordance with the present invention, it is preferable to provide partitions between regions of varying flow rate where the controlling characteristic, such as thickness of a pipe wall, changes abruptly. By way of example, when quenching upset pipe a partition is preferably located at each boundary of the upset to ensure a relatively clear line of demarcation in the cooling regimes between the upset and the adjacent segment of the pipe.

A cross sectional view of an exterior quenching compartment is shown in Figure 5. A series of flow chamber walls 71 serve to divide the annulus 36 created by walls 34 and 35 into flow chambers 73. The flow chambers 73 are equipped with a series of L-shaped deflector plates 72 having a plurality of inlets 74. The deflector plates run along the length of each flow chamber 73. They are substantially parallel to the pipe and angled in such a fashion that a cooling medium passing through openings or slots 74 in the wall of each deflector plate is directed around a segment of pipe 130. Openings or slots 74 are preferably arranged such that a cooling medium from pipes 55, 56 and 57 is also directed in a swirling motion. Thus, the series of deflector plates 72 are so arranged in each flow chamber 73 surrounding pipe 130 that the swirling cooling medium flows in a circumferential pattern about the exterior surface of the pipe 130. Wall 35 is provided with appropriate openings or cutout portions to accommodate the flow from the deflectors.

Interior wall 35 may also be provided with a plurality of threaded holes which place flow chambers 73 in communication with the interior of the receptacle 30. Nozzles may then be inserted in the threaded holes to direct the cooling medium from each flow chamber 73 in a circumferential flow pattern around the exterior surface of the pipe. As the holes may be filled with plugs, the number, as well as the type of nozzles, may be varied depending upon the specific flow pattern desired.

As another alternative, wall 35 may be provided with a series of openings, or slots as in Figure 6 which are angled to properly direct the flow of the cooling medium around the pipe.

In accordance with the present invention, the arrangement of the deflector plates, nozzles or openings must be such as to provide a circumferential flow pattern of the cooling medium around the exterior of the pipe 130. The cooling medium is preferably directed so as to not im-. pinge upon the pipe surface in order to facilitate uniform cooling of the pipe. As indicated in Figure 6, a curved deflector plate 141 may also be provided to aid in completion of the circumferential flow pattern about the upper portion of pipe 130. A hydraulic cylinder and piston mechanism shown generally at 142 may be provided to move the flexible plate out of the path of the pipe 130 as it enters receptacle 30 from ramp 23. As shown, the upper deflector plate 141 could be pivotally attached to interior wall 35 so as to form a continuation of wall 35 extending out and over the central axis of receptacle 30. Hydraulic cylinder and piston mechanism 142 could be attached to a shaft 144 by means of a series of flanges 143 such that retraction of the piston would cause upward and outward movement of the deflector plate 141.

Ribs or quenching supports 31 are adapted to closely conform to the lower circumference of the pipe 130 as it rests on each rib. Additionally, each of the upper segments of the quenching supports is adapted to facilitate movement of a pipe in and out of the receptacle.

As the type of rib or quenching support may differ along the length of the receptacle 30, pipes of varying sizes and diameters may be accommodated. Additionally, any given quenching support or rib may be readily detached by removal of the pins 38 and replaced with a different quenching support or rib. Thus, the system may be adapted to handle varying sizes of pipe with variable circumferences along their length.

By way of example, the ribs closer to the center may accommodate a pipe with an outside diameter of 5 inches (12.7 cm) while ribs able to accommodate a pipe with an outside diameter of 5.875 inches (14.9 cm), may be inserted at the end of the receptacle. Thus, 5 inch (12.7 cm) pipe with an external upset of 5.875 inches (14.9 cm) may be secured along its length within the receptacle 30.

It may be preferable in some instances to provide different size receptacles 30 to accommodate varying ranges of pipe. For example, one unit might have a receptacle adaptable to accept pipe with outside diameters of 4.5 to 14 inches, while a smaller unit might be adaptable to accept pipe ranging from 1.5 to 4.5 inches in outside diameter.

Referring now to Figure 8, the internal quencher 80 comprises a cooling medium feed conduit 81 and a gas feed conduit 82 mounted in cylindrical rod 87. Cooling medium feed conduit 81 is mounted in frame 93 and is equipped with an internal fixed sleeve 181, which is integrally mated to the interior wall of conduit 81. Movable sleeve 182, which has a tapered end portion 94, is telescopically mated with the internal sleeve 181. The tapered end portion 94 is adapted to sealingly engage the inlet of pipe 130.

It is preferable that vanes 182 remain essentially stationary. For example, when the vanes are integrally mounted in movable sleeve 182, the sleeve should be mounted to avoid substantial rotation of the vanes by the swirling cooling medium passing through the sleeve. By way of example, the sleeve 181 could be fitted with grooves to accept flanges extending from movable sleeve 182.

Cylindrical rod 87 is integrally mounted in movable sleeve 182 by means of helical vanes 84, which are integrally attached along the interior surface of sleeve 182. As shown in Figure 9 cylindrical rod 87 is also supported by rods 83 which are mated into sliding tube 182.

The gas feed conduit 82 is connected to conduit 89 such that the flow of gas through conduit 82 may be controlled by shut off valve 88. Gas feed conduit 82 is supported by cylindrical rod 87 along its length. Cylindrical rod 87 is telescopically mated into sealed housing or stuffing box 89 which is attached at one end to piston 86. Thus, movement of piston 86 causes the movement of rod 87 and hence conduit 82 and sleeve 182. Conduit 89 is attached to a flexible hose 150 to accommodate movement of the gas feed conduit 82 with cylindrical rod 87.

The outlet of gas feed conduit 82 is equipped with a plug or nozzle 90 which is shown in more detail in Figure 10. The plug 90 is threaded into cylindrical rod 87 by means of threads shown at 92. As the end of feed conduit 82 is equipped with apertures 91 the flow of gas through conduit 82 occurs around the tapered end portion of plug 90 as shown by the arrows in Figure 10.

In accordance with the present invention, the spiral vanes are preferably at an angle of approximately 35 degrees with the horizontal, particularly when water is used as a cooling medium. This angle will impart a relatively long spiral to the flowing water and so reduce the time the water travels the length of the pipe. Additionally, multiple vanes are preferred in order to aid in imparting sufficient turbulence to the cooling medium. However, the arrangement of the vanes may be varied depending upon the exact nature of the helical motion desired in the cooling medium. For example, variations in the type and amount of cooling medium, the type of pipe being quenched, the severity of the quench desired and the amount of gas to be injected may all affect the exact configuration chosen for the vanes.

A clamp indicated generally at 100 is provided to hold the pipe 130 in place. The clamp comprises an arm 101 and a clamping member 108. Although not shown, the lower portion of clamping member 108 is contoured to engage the upper surface of pipe 130 when horizontal arm 101 is lowered into the position shown in Figure 2. Arm 101 is rotatably mounted on clamp base 107 by means of pin 104. Piston 102 of hydraulic cylinder 103 is attached by means of pin 105 to flange 106. As flange 106 is integrally mounted on arm 101 the movement of piston 102 causes the upward movement of arm 101. The movement of piston 102 and arm 101 is further facilitated by the pivotal mounting of hydraulic cylinder 103 onto flange 110 by means of pin 111. As shown in Figure 8, hydraulic cylinder 103 is mounted on base 109 which rests on the top of frame 93.

Referring again to Figures 1-10, in operation a steel pipe 130 is heated to a temperature sufficiently above its austenizing temperature to avoid cooling below its critical transformation temperature prior to entering the receptacle. The pipe is then placed in a position substantially parallel to receptacle 30 by means of feed rolls 11. Piston 18 of hydraulic cylinder 17 is then retracted causing angular feed arms 22 to rotate about shaft 21 such that the arcuate portion 24 of each angular feed arm 22 comes into contact with and cradles the underside of pipe 130 at various points along its length. The pipe 130 is then lifted by angular feed arms 22 onto feed ramp 23, whereupon the pipe 130 rolls down quenching support 31 and into the lower portion of pipe receptacle 30.

While the pipe 130 is being moved into position on feed rolls 11, the cooling medium source 50 fills receptacle 30 with water. Thus, as the hot pipe rolls into the pipe receptacle 30, its fall is cushioned by the water as it is received by ribs or contoured pipe supports 31 which are adapted to cradle the lower portion of the pipe. As the diameter of the ribs may be varied along the length of receptacle 30, pipe of varying diameter or size may be cradled along its length and rest securely in arcuate portions 34 of each quenching support.

Once the pipe is resting in receptacle 30, hydraulic cylinder 103 is activated and piston 102 extended, thus causing arm 101 to lower into a horizontal position as it rotates about pin 104. This in turn brings the lower contoured portion of clamping member 108 into contact with the upper portion of pipe 130. By means of hydraulic cylinder 103, piston 102 and arm 101, clamping member 108 exerts a downward force on the end of the cradled pipe 130. As the pipe is cradled into arcuate sections 34 and clamping member 108 is contoured to the upper surface of the pipe, only one clamping member is needed to substantially hold the pipe in place against the force of the cooling medium as it impacts the pipe 130. The clamp 100 also serves to hold the pipe in place against the movement of tapered end portion 94 of sleeve 182.

As the pipe 130 is being clamped into place by means of clamp 100, cylinder rod 87 and hence feed gas conduit 82, is moved forward by hydraulic cylinder 85 and piston 86. The movement of cylindrical rod 87 through sealed housing or stuffing box 89 in turn causes the forward movement of movable sleeve 84. As the movable sleeve 84 travels forward toward the inlet of pipe 130 it slides through fixed sleeve 181 until the tapered end segment 94 sealingly engages the inlet of pipe 130 as shown in Figure 8.

Once the pipe is thus positioned and the internal quencher 80 is brought into contact with the pipe inlet, water is fed through feed conduit 81. Concurrently therewith valves 52 are opened to deliver the water through deflector plates 72 or appropriately placed nozzles and hence in a circumferential flow pattern around the exterior of pipe 130, while shut off valve 88 is opened to allow gas from flexible conduit 150 to pass through conduit 89 and gas feed conduit 82 and hence into the water passing through tapered end portion 94 of sleeve 182. As the water must pass through helical vanes 84, the water enters the inlet of pipe 130 in a helical flow pattern. Additionally, the water is injected with a sufficient amount of gas, such as air, to aerate the water and insure sufficient turbulence to avoid the creation of steam and vapor pockets and so prevent nonuniform cooling and otherwise facilitate heat transfer from the pipe wall into the water.

In accordance with one aspect of the present invention, the internal and external quenches preferably begin almost simultaneously in order to promote a more uniform cooling sequence across the thickness of the pipe wall. Thus, the circumferential flow of water from the flow chamber 73 and inlet 94 preferably begins within a few tenths of a second or less after the pipe 131 is rolled into receptacle 30. Additionally, the flow of waterfrom flow chambers 73 may begin before the pipe leaves feed rolls 11. In this regard it is noted that the continual replenishment of the water serves to remove impurities and maintain the water temperature at the desired level.

In accordance with the present invention, it is important to maintain the flow from deflector plates 72 into each of the exterior quenching compartments formed by member 32 and movable arm 33 in a substantially circumferential pattern such that the flow of water moves along the exterior surface of the pipe 130. The water should generally not directly impinge on the pipe if uniform cooling is to be achieved.

The pressure of the water entering from valves 52 should be sufficient to create sufficient turbulence so that pockets of steam or vapor are removed as the water flows circumferentially along the pipe surface. Additionally, the flow rate should be such as to provide a fairly rapid turnover of the water in each compartment in order to prevent the circumferentially flowing turbulent water within each compartment from rising above a specified temperature. More particularly, the flow rate is preferably such as to keep the water at an overall temperature of about 80°F (27°C) and preferably 70°F (21°C) or less, since the cooling power of water increases rapidly as water temperature increases beyond about 75°F (24°C). In fact, this loss of cooling power is almost expotential such that water at a temperature of 120°F (49°C) has only about 20% of the cooling power of water at 70°F (21°C). However, use of water at a higher temperature can still prove advantageous when compared to prior art processes using water of a similar temperature due to the favorable circumferential flow pattern created by the deflector plates and the high turnover of the water in each compartment.

Other mechanisms, such as conduits placed in receptacle 30, may be provided in place of the difference in receptacle wall height to facilitate the appropriate replenishment of the cooling medium. However, as indicated, the mechanism should be able to provide sufficient turnover of the cooling medium to properly control temperature.

The water flowing into the interior of the pipe is preferably at a pressure of about 100 psi and should be within the range of about 60 to 110 psi prior to injection of the gas. This is believed to be a high enough pressure to provide needed turbulence and allow the gas to force the water to adhere more closely to the interior pipe wall as it passes through the pipe.

The internal and external quenches are continued for a predetermined amount of time. The time of the quench, the rate of flow of the cooling medium through flow chambers 73 and cooling medium feed conduit 81, and the flow of gas through gas feed conduit 82 may all be regulated during the quenching operation to provide a proper cooling sequence for the pipe 130. To this end thermocouples and other sensors (not shown) may be employed along with appropriate process controls to control the flow of the cooling medium and gas in order to control the cooling sequence undergone by the pipe.

Upon completion of the cooling sequence hydraulic cylinder 43 retracts piston 46 thus causing movable support 49 and integrally mounted movable arm 33 to rotate about shaft 38. As the arcuate section 34 of movable arm cradles lower portion of pipe 130, pipe 130 is lifted up out of the receptacle 30 and onto ramp 41. The quenched pipe then rolls down ramp 41 and onto rollers 39 where it may be forwarded for further processing, such as tempering.

As will be appreciated by one skilled in the art having the benefit of this disclosure, given the variable flow rates and the other conditions attainable in each compartment, the present invention is particularly suitable for quenching internal and external upset pipe, casing or tapered steel pieces. Of course, in the case of pipe with uniform thickness the flow rates do not necessarily have to be varied. Additionally, steel pipe with walls of greater thickness or lower alloy content may now be successfully heat treated.

The process and apparatus of the present invention may also be used to treat tool joints after they are welded to a tubular member such as drill pipe. Thus, the tool joint and pipe may be of similar composition and the tool joint need not have a higher alloy content to withstand the temperature changes caused by welding. For example, a tool joint, which may be thought of as a sleeve of additional thickness added to the end of a pipe, may first be welded to a piece of pipe. Thereafter, the pipe-tool joint combination may be heated above its critical austenizing temperature and quenched in accordance with the present invention.

As will be appreciated by one skilled in the art having the benefit of this disclosure a number of modifications may be made to the foregoing apparatus and method within the spirit of the present invention. For example, receptacle 30 may be varied in shape and the number of flow chambers and deflector plates may be varied depending on the source of the cooling medium, the maximum and minimum thickness of pipe or other object to be quenched by a given unit and other variables. Additionally, although the cooling medium is preferably water and the gas is preferably air, any variety of cooling media or gases may be employed or interchanged within the spirit of the present invention. Furthermore, the interior quenching means 80 may be used with conventional quenching techniques. Similarly, the exterior quenching means 70 may be used to quench the exterior of the pipe while conventional quenching techniques are used on the interior. However, it is preferable in most cases to use both in order to facilitate uniform and rapid heat transfer from the pipe to the cooling medium and otherwise take full advantage of the present invention. Also the nature and extent of the partitions created by movable arm 33 and fixed member 32 or the number of compartments may be varied depending upon the cooling sequence or other effects desired along segments of the pipe.

Further modifications and alternative embodiments of the apparatus and method of this invention will be apparent to those skilled in the art in view of this description. Accordingly, this description is to be construed as illustrative only and is for the purpose of teaching those skilled in the art the manner of carrying out the invention. It is to be understood that the forms of the invention herewith shown and described will be taken as the presently preferred embodiments. Various changes may be made in size, shape and arrangement of parts. For example, equivalent elements or materials may be substituted for those illustrated and described herein, parts may be reversed, and certain features of the invention may be utilized independent of the use of other features, all of which would be apparent to one skilled in the art after having the benefit of this description of the invention.

## Claims

1. An apparatus for quenching a piece of steel in a receptacle (30) adapted to receive the piece of steel of the type comprising a cooling medium source (50) for supplying a cooling medium to the receptacle (30), said cooling medium source (50) comprising an exterior quenching means (70), characterized in that said exterior quenching means is in communication with the interior of the receptacle (30) through a plurality of openings in the receptacle (30) and adapted for separately directing a cooling medium in a substantially circumferential flow pattern at variable flow rates around separate exterior segments of the piece of steel as the piece of steel is held in the receptacle (30), said receptacle (30) being configured to permit sufficient turnover of cooling medium to replenish at least a portion of the cooling medium directed in the circumferential flow pattern once such portion of the cooling medium has removed heat from the piece of steel.

2. The apparatus of claim 1 further characterized in that the receptacle (30) is longitudinally divided into compartments to facilitate a rate of cooling variable among exterior segments of the steel piece.

3. The apparatus of claim 1 further characterized in that the receptacle (30) is adapted to receive a steel pipe of varying diameter.

4. The apparatus of claim 1 further characterized in that the steel piece rests on partitions mounted along the interior of the receptacle (30).

5. The apparatus of claim 4 further characterized in that the partitions are contoured to fit the exterior surface of the steel piece.

6. The apparatus of claim 1 wherein the piece of steel is a hollow-bodied steel piece with an opening at each end thereof and further characterized in that there is provided internal quenching means (80) for supplying a cooling medium to the interior of the hollow-bodied steel piece while it is held in the receptacle (30).

7. The apparatus of claim 6 further characterized in that the internal quenching means (80) comprises a means for passing a cooling medium through the interior of the steel piece and a gas injection conduit (82) for injecting a gas into the cooling medium to insure sufficient turbulence in the cooling medium as it passes through the interior of the steel piece to facilitate heat transfer from the interior surface of the steel piece to the cooling medium.

8. The apparatus of claim 6 wherein the hollowed-bodied steel piece is a pipe (130) and further characterized in that the interior quenching means (80) includes
a cooling medium conduit (81) located along the axis of the pipe (130) and having a tapered outlet (94) adapted to direct the cooling medium into the interior of the pipe (130);
a gas conduit (82) telescopically mated in the cooling medium conduit (81) and having a gas conduit outlet near the tapered outlet (94) of the cooling medium conduit (81), the gas conduit outlet being adapted to inject a gas from the gas conduit (82) into the cooling medium; and
a series of helical vanes (84) mounted in the interior of the cooling medium conduit (81) and adapted to impact a helical flow pattern to the cooling medium leaving the tapered outlet (94).

9. The apparatus of claim 1 further characterized in that one side of the receptacle (30) is lower than the other side to thereby facilitate the rapid exchange of cooling medium.

10. The apparatus of claim 1 wherein the steel piece is a pipe and further characterized in that the receptacle (30) has a curved wall (134) with a plurality of openings and one or more supports (49) along the length of the receptacle (30), said supports being at least partially contoured to engage a portion of the pipe (130) placed in the receptacle (30) and portion the interior of the receptacle (30) along its length into segments and said curved wall (134) being configured to form a generally annular space around a portion of the pipe (130); and that there are provided:
a pressurized source (50) of cooling medium in communication with the receptable (30) through the plurality of openings, the pressurized source (50) being configured in conjunction with the openings and the curved wall to provide a generally circumferential flow pattern of the cooling medium around the pipe (130) in the receptacle and the pressurized source and said curved wall being further configured to facilitate a rapid exchange of cooling medium sufficient to replenish at least a portion of the cooling medium directed in the circumferential flow pattern once such cooling medium has removed heat from the pipe (130); and
an interior quenching means (80) operatively connected to the receptacle (30) for passing a cooling medium through the interior of the pipe (130) and. including a cooling medium conduit (81) adapted to direct a cooling through the interior of the pipe (130) independently of cooling medium passing around the exterior of the pipe (130).

11. The apparatus of claim 10 further characterized in that there is provided:
at least one flow chamber (73) mounted on an exterior surface of the receptacle (30) in communication with a plurality of the openings; and
a plurality of deflectors (72) mounted on each flow chamber (73) and configured to direct the cooling medium through the receptacle openings (74) in a circumferential flow pattern around the surface of the pipe (130).

12. A method of heat treating pieces of steel including the step of heating each piece of steel to a temperature above its austenizing temperature, wherein is accomplished the step of:
supplying a sufficient amount of continually replenished cooling medium to a receptacle (30) to quench the piece of steel in the receptacle (30) prior to removing the piece of steel while distributing at least a portion of the cooling medium including a portion of the continually replenished cooling medium in a substantially circumferential flow pattern around the steel piece while it is in the receptacle to reduce the temperature increase in the cooling medium that results from heat removal from the steel piece, said flow pattern being capable of sufficient variation among finite longitudinal segments of the steel piece to facilitate proper transformation of the steel along the length of the piece of steel.

13. The method of claim 12 wherein the piece of steel is a steel pipe (130) and further characterized in that there is provided the step of substantially concurrently with circuiting the cooling medium around exterior segments of the pipe (130), directing a cooling medium through the interior of the pipe (130) at a flow rate which may be independently varied from the circumferential flow rate of the cooling medium around one or more exterior segments of the pipe (130).

14. The method of claim 13 further characterized in that a gas is injected into the cooling medium directed through the interior of the pipe (130).

15. The method of claims 13 or 14 further characterized in that the cooling medium is directed through the. interior of the pipe (130) in a helical flow pattern.

16. The method of claim 12 further characterized in that the cooling medium comprises water maintained at a temperature of 80°F (27°C) or less.

17. The method of claim 12 further characterized in that the cooling medium comprises water maintained at a pressure in the range of approximately 80 to 130 psi (about 5.5 to 9 bar).

## Patentansprüche

1. Vorrichtung zum Abschrecken eines Stückes Stahl in einem Behälter (30) zur Aufnahme des Stückes Stahl, der eine Kühlmittelquelle (50) zur Förderung eines Kühlmittels zum Behälter (30) aufweist, wobei die Kühlmittelquelle (50) eine äußere Abschreckeinrichtung (70) aufweist, dadurch gekennzeichnet, daß die äußere Abschreckeinrichtung mit dem Inneren des Behälters (30) über eine Mehrzahl von Öffnungen im Behälter (30) in Verbindung steht und zur getrennten Zufuhr eines Kühlmediums in einem im wesentlichen in Umfangsrichtung verlaufenden Strömungsmuster mit variablen Strömungsgeschwindigkeiten um separate Abschnitte der Außenseite des Rohrs herum vorgesehen ist, wenn das Stück Stahl im Behälter (30) gehalten wird, wobei der Behälter (30) derart ausgebildet ist, daß eine ausreichende Umwälzung des Kühlmediums ermöglicht wird, um wenigstens einen Teil des Kühlmediums, der in das umfangsseitige Strömungsmuster gerichtet ist, nachzufüllen bzw. aufzufrischen, sobald dieser Teil des Kühlmediums Wärme aus dem Stück Stahl entfernt hat.

2. Vorrichtung nach Anspruch 1, weiterhin dadurch gekennzeichnet, daß der Behälter (30) in Längsrichtung in Abschnitte unterteilt ist, um eine über die Abschnitte der Außenseite variable Abkühlgeschwindigkeit zu ermöglichen.

3. Vorrichtung nach Anspruch 1, weiterhin dadurch gekennzeichnet, daß der Behälter (30) zur Aufnahme eines Stahlrohres mit variierendem Durchmesser eingerichtet ist.

4. Vorrichtung nach Anspruch 1, dadurch gekennzeichnet, daß das Stück Stahl auf entlang dem Inneren des Behälters angeordneten Trennwänden ruht.

5. Vorrichtung nach Anspruch 4, dadurch gekennzeichnet, daß die Kontur der Trennwände der Außenfläche des Stückes Stahl angepaßt ist.

6. Vorrichtung nach Anspruch 1, wobei das Stück Stahl ein Stück Stahl mit hohlem Körper mit einer Öffnung an jedem Ende ist, und weiterhin dadurch gekennzeichnet, daß eine innere Abschreckeinrichtung (80) zum Fördern von Kühlmedium zum Inneren des mit dem hohlen Körper versehenen Stahlstückes vorgesehen ist, während dieses im Behälter (30) angeordnet ist.

7. Vorrichtung nach Anspruch 6, dadurch gekennzeichnet, daß die innere Abschreckeinrichtung (80) eine Einrichtung zum Hindurchleiten eines Kühlmediums durch das Innere des Stahlstückes und eine Gaseinblasleitung (82) zum Einblasen eines Gases in das Kühlmedium aufweist, um eine genügende Turbulenz im Kühlmedium bei dessen Durchgang durch das Innere des Stahlstückes zu gewährleisten und damit die Wärmeübertragung von der Innenfläche des Stahlstückes auf das Kühlmedium zu erleichtern.

8. Vorrichtung nach Anspruch 6, wobei das mit dem hohlen Körper versehene Stahlstück ein Rohr (130) ist, dadurch gekennzeichnet, daß die innere Abschreckeinrichtung (80) folgende Teile aufweist:
eine Kühlmittelleitung (81), die entlang der Achse des Rohres (130) angeordnet ist und einen verjüngten Auslaß (94) aufweist und zum Einleiten des Kühlmediums in das Innere des Rohres (130) vorgesehen ist;
eine Gasleitung (82), die teleskopartig in der Kühlmediumleitung (81) angeordnet ist und einen Gasleitungsauslaß nahe dem sich verjüngenden Auslaß (94) der Kühlmediumleitung (81) aufweist, wobei der Gasleitungsauslaß zum Einblasen eines Gases von der Gasleitung (81) in das Kühlmedium vorgesehen ist; und
eine Reihe von im Inneren der Kühlmittelleitung angeordneten, entlang Schraubenlinien ausgerichteten Leitschaufeln zum Erzeugen eines schraubenförmigen Strömungsmusters in dem aus dem sich verjüngenden Aulaß (94) austretenden Kühlmedium.

9. Vorrichtung nach Anspruch 1, dadurch gekennzeichnet, daß eine Seite des Behälters (30) niedriger ist als die andere Seite, um damit den schnellen Austausch des Kühlmediums zu erleichtern.

10. Vorrichtung nach Anspruch 1, wobei das Stahlstück eine Rohr ist, dadurch gekennzeichnet, daß der Behälter (30) eine gekrümmte Wand (134) mit einer Mehrzahl von Öffnungen und einer oder mehreren Stützen (49) entlang der Länge des Behälters (30) aufweist, wobei die Stützen wenigstens teilweise derart geformt sind, daß sie an einem Bereich des Rohres (130) anliegen, das im Behälter (30) angeordnet ist, und das Innere des Behälters (30) entlang seiner Länge in Segmente unterteilen, und wobei die gekrümmte Wand (134) derart ausgebildet ist, daß sie einen im wesentlichen ringförmigen Raum um einen Teil des Rohres (130) bildet, und daß folgende Teile vorgesehen sind:
eine unter Druck stehende Quelle (50) von Kühlmedium, die über eine Mehrzahl von Öffnungen in Verbindung mit dem Behälter (30) steht, wobei die Druckquelle (50) in Verbindung mit den Öffnungen und der gekrümmten Wand so ausgebildet ist, daß ein im wesentlichen umfangsseitiges Strömungsmuster des Kühlmediums um das Rohr (130) im Behälter geformt wird, und wobei die Druckquelle und die gekrümmte Wand ferner so ausgebildet sind, daß ein schneller Austausch des Kühlmediums erleichtert wird, um ausreichend wenigstens einen Teil des Kühlmediums, das in das umfangsseitige Strömungsmuster ausgerichtet ist, wieder aufzufüllen, wenn das Kühlmedium Wärme aus dem Rohr (130) entfernt hat, und
eine Innere Abschreckeinrichtung (80), die in Wirkverbindung mit dem Behälter (30) zum Hindurchleiten eines Kühlmediums durch das Innere des Rohres (130) steht und eine Kühlmediumleitung (81) aufweist, die ein Kühlmedium durch das Innere des Rohres (130) unabhängig von dem Kühlmedium, das um das Äußere des Rohres (130) herumfließt, hindurchleitet.

11. Vorrichtung nach Anspruch 10, dadurch gekennzeichnet, daß wenigstens eine Durchflußkammer (73), die an der Außenfläche des Behälters (30) in Verbindung mit einer Mehrzahl von Öffnungen angeordnet ist, und eine Mehrzahl von Leitschaufeln (72) vorgesehen ist, die an jeder Durchflußkammer (73) angeordnet sind und zur Ausrichtung des Kühlmediums durch die Behälteröffnungen (74) in einem umfangsseitigen Flußmuster um die Fläche des Rohres (130) ausgebildet sind.

12. Verfahren zur Wärmebehandlung von Stahlstücken, welches den Verfahrensschritt des Erwärmens jeden Stahlstückes auf eine Temperatur oberhalb seiner Austenittemperatur umfaßt, wobei der folgende Verfahrensschritt ausgeführt wird:
Fördern einer genügenden Menge von kontinuierlich nachgefülltem Kühlmedium zu einem Behälter (30), um das Stahlstück im Behälter (30) vor dem Entfernen des Stahlstückes abzukühlen, während wenigstens ein Teil des Kühlmediums mit einem Teil des kontinuierlich nachgefüllten Kühlmediums in ein im wesentlichen umfangsseitiges Flußmuster um das Stahlstück herum verteilt wird, während es sich im Behälter befindet, um den Temperaturanstieg im Kühlmedium zu vermindern, welcher aus der Wärmeabfuhr von dem Stahlstück resultiert, wobei das Strömungsmuster dazu in der Lage ist, eine ausreichende Veränderung unter finiten Längssegmenten des Stahlstückes zu erreichen, um eine korrekte Transformation des Stahles entlang der Länge des Stahlstückes zu erleichtern.

13. Verfahren nach Anspruch 12, wobei das Stück Stahl ein Stahlrohr (130) ist, gekennzeichnet durch den Verfahrensschritt des im wesentlichen gleichzeitig mit dem Zirkulieren des Kühlmediums um äußere Bereiche des Stahlrohres (130) Richtens eines Kühlmediums durch das Innere des Rohres (130) mit einer Flußgeschwindigkeit, welche unabhängig von der umfangsseitigen Flußgeschwindigkeit des Kühlmediums um ein oder mehrere äußere Segmente des Rohres (130) variiert werden kann.

14. Vorrichtung nach Anspruch 13, dadurch gekennzeichnet, daß ein Gas in das Kühlmedium eingeblasen wird, das durch das Innere des Rohres (130) geleitet wird.

15. Verfahren nach Anspruch 13 oder 14, dadurch gekennzeichnet, daß das Kühlmedium durch das Innere des Rohres (130) in einem schraubenartig ausgerichteten Flußmuster geleitet wird.

16. Verfahren nach Anspruch 12, dadurch gekennzeichnet, daß das Kühlmedium Wasser ist, das bei einer Temperatur von 80°F (27°C) oder weniger gehalten wird.

17. Verfahren nach Anspruch 12, dadurch gekennzeichnet, daß das Kühlmedium Wasser ist und bei einem Druck im Bereich von ungefähr 80 bis 130 psi (ungefähr 5,5 bis 9 bar) gehalten wird.

## Revendications

1. Appareil pour tremper une pièce d'acier dans un réceptacle (30) adapté pour recevoir la pièce d'acier du type comprenant une source de fluide de refroidissement (50) destinée à appliquer un fluide de refroidissement dans le réceptacle (30), ladite source de fluide de refroidissement (50) comportant un moyen extérieur de trempe (70), caractérisé par le fait que ledit moyen extérieur de trempe est en communication avec l'intérieur du réceptacle (30) grâce à une pluralité d'ouvertures ménagées dans le réceptacle (30) et adaptées pour orienter séparément un fluide de refroidissement selon une répartition d'écoulement sensiblement circonférentielle avec des vitesses d'écoulement variable autour de segments extérieurs distincts de la pièce d'acier quand la pièce d'acier est maintenue dans le réceptacle (30), ledit réceptacle (30) ayant une configuration qui permet une rotation suffisante du fluide de refroidissement pour remplacer au moins une partie du fluide de refroidissement orienté selon la répartition d'écoulement circonférentielle lorsqu'une telle portion du fluide de refroidissement a retiré la chaleur de la pièce d'acier.

2. Appareil selon la revendication 1, caractérisé en outre par le fait que le réceptacle (30) est divisé dans la direction longitudinale en compartiments afin de faciliter l'établissement d'un taux de refroidissement variable parmi les segments extérieurs de la pièce d'acier.

3. Appareil selon la revendication 1, caractérisé en outre par le fait que le réceptacle (30) est adapté à recevoir un tuyau d'acier de diamètre variable.

4. Appareil selon la revendication 1, caractérisé en outre par le fait que la pièce d'acier repose sur des cloisons montées le long de l'intérieur du réceptacle (30).

5. Appareil selon la revendication 4, caractérisé en outre par le fait que les cloisons ont une conformation qui s'adapte à la surface extérieure de la pièce d'acier.

6. Appareil selon la revendication 1 dans lequel la pièce d'acier est une pièce d'acier à corps creux avec une ouverture à chaque extrémité et caractérisé en outre par le fait qu'il est prévu un moyen interne de trempe (80) afin d'appliquer unfluide de refroidissement à l'intérieur de la pièce d'acier à corps creux pendant que cette pièce est maintenue dans le réceptacle (30).

7. Appareil selon la revendication 6, caractérisé en outre par le fait que le moyen interne de trempe (80) comprend un moyen pour faire passer un fluide de refroidissement par l'intérieur de la pièce d'acier et un conduit d'injection d'un gaz

(82) pour injecter un gaz dans le fluide de refroidissement afin de communiquer au fluide de refroidissement pendant son passage à l'intérieur de la pièce d'acier, une turbulence suffisante pour faciliter le transfert de chaleur entre la surface intérieure de la pièce d:acier et le fluide de refroidissement.

8. Appareil selon la revendication 6 dans lequel la pièce d'acier à corps creux est un tuyau (130) et caractérisé en outre par le fait que le moyen intérieur de trempe (80) comprend:
- un conduit de fluide de refroidissement (81) placé le long de l'axe du tuyau (130) et ayant une sortie conique (84) adaptée à orienter le fluide de refroidissement vers l'intérieur du tuyau (130);
- un conduit de gaz (82) adapté par un système télescopique dans le conduit du fluide de refroidissement (81) et possédant une sortie de conduit de gaz à proximité de la sortie conique (94) du conduit du fluide de refroidissement (81), la sortie du conduit de gaz étant adaptée à injecter un gaz provenant du conduit de gaz (82) dans le fluide de refroidissement; et
- une série de déflecteurs hélicoïdaux (83) montés à l'intérieur du conduit du fluide de refroidissement (81) et adaptés à communiquer une répartition hélicoïdale d'écoulement au fluide de refroidissement quittant la sortie conique (94).

9. Appareil selon la revendication 1, caractérisé en outre par le fait qu'un côté du réceptacle (30) est plus bas que l'autre côté afin de faciliter ainsi l'échange rapide du fluide de refroidissement.

10. Appareil selon la revendication 1, dans lequel la pièce d'acier est un tuyau, et caractérisé en outre par le fait que le réceptacle (30) comprend une paroi (134) courbée avec une pluralité d'ouvertures et un ou plusieurs supports (49) répartis sur la longueur du réceptacle (30), lesdits supports étant au moins partiellement conformés pour venir en contact avec une portion du tuyau (130) placé dans le réceptacle (30) et pour subdiviser l'intérieur du réceptacle (30) sur sa longueur en segments et ladite paroi courbe (134) étant configurée pour délimiter un espace généralement annulaire autour d'une portion du tuyau (130); et par le fait qu'il est prévu:
- une source pressurisée (50) de fluide de refroidissement en communication avec le réceptacle (30) grâce à la pluralité d'ouvertures, la source pressurisée (50) étant configurée en liaison avec les ouvertures et la paroi courbe pour créer une répartition d'écoulement sensiblement circonférentielle du fluide de refroidissement autour du tuyau (130) placé dans le réceptacle, et la source sous pression ainsi que ladite paroi courbe étant encore configurées pour faciliter un échange rapide et suffisant du fluide de refroidissement pour reconstituer au moins une portion du fluide de refroidissement orientée selon une configuration d'écoulement circonférentielle une fois que ce milieu de refroidissement a éliminé la chaleur du tuyau (130), et
- un moyen intérieur de trempe (80) fonctionnellement connecté au réceptacle (30) pour faire passer un fluide de refroidissement à travers l'intérieur du tuyau (130) et comprenant un conduit à fluide de refroidissement (81) adapté à orienter un fluide de refroidissement à l'intérieur du tuyau (130) indépendamment du fluide de refroidissement passant sur l'extérieur du tuyau (130).

11. Appareil selon la revendication 10, caractérisé en outre par le fait qu'il est prévu:
- au moins une chambre de circulation (73) installée sur la surface extérieure du réceptacle (30) en communication avec une pluralité d'ouvertures; et
- une pluralité de déflecteurs (72) montés sur chaque chambre d'écoulement (73) et configurés pour orienter le fluide de refroidissement à travers les ouvertures de réceptacle (74) selon une répartition circonférentielle d'écoulement autour de la surface du tuyau (130).

12. Procédé de traitement à chaud de pièces d'acier comprenant l'opération de chauffage de chaque pièce d'acier jusqu'à une température dépassant sa température d'austénisation dans lequel l'opération suivante est effectuée:
- application d'une quantité.suffisante d'un fluide de refroidissement dont la quantité est rétablie en permanence, à un réceptacle (30) pour tremper la pièce d'acier située dans le réceptacle (30) avant de retirer la pièce d'acier tout en répartissant au moins une partie du fluide de refroidissement y compris une partie du fluide de refroidissement ajoutée en permanence selon une répartition d'écoulement sensiblement circonférentielle autour de la pièce d'acier pendant que cette dernière se trouve dans le réceptacle afin de réduire l'augmentation de température du milieu de refroidissement qui résulterait de la chaleur retirée à la pièce d'acier, ladite répartition d'écoulement étant capable d'une variation suffisante parmi des segments longitudinaux finis de la pièce d'acier pour faciliter une transformation convenable de l'acier sur la longueur de la pièce d'acier.

13. Procédé selon la revendication 12 dans lequel la pièce d'acier est un tuyau d'acier (130) et caractérisé en outre par le fait qu'il est prévu l'opération sensiblement simultanée à la mise en circulation du fluide de refroidissement autour des segments extérieurs du tuyau (130), d'orientation d'un fluide de refroidissement traversant l'intérieur du tuyau (130) avec une vitesse d'écoulement qui peut être modifiée de façon indépendante de la vitesse circonférentielle d'écoulement du fluide de refroidissement autour d'un ou plusieurs des segments extérieurs du tuyau (130).

14. Procédé selon la revendication 13, caractérisé en outre par le fait qu'un gaz est injecté dans le fluide de refroidissement orienté vers l'intérieur du tuyau (130).

15. Procédé selon l'une des revendications 13 ou 14, caractérisé en outre par le fait que le fluide de refroidissement est orienté vers l'intérieur du tuyau (130) .selon une répartition d'écoulement hélicoïdale.

16. Procédé selon la revendication 12, caractérisé en outre par le fait que le fluide de refroidissement est constitué par de l'eau maintenue à une température de 27°C (80°F) ou moins.

17. Procédé selon la revendication 12, caractérisé en outre par le fait que le fluide de refroidissement contient de l'eau maintenue sous une pression située dans la gamme allant d'environ 5,5 à 9 bars (80 à 130 psi).
